

## UNITED STATES PATENT OFFICE

ERNST TEUPEL, OF DORMAGEN, GERMANY, ASSIGNOR TO I. G. FARBENINDUSTRIE AKTIENGESELLSCHAFT, OF FRANKFORT-ON-THE-MAIN, GERMANY, A CORPORATION OF GERMANY

## ALKYL-ARALKYL-CELLULOSE ESTERS AND PROCESS OF MAKING THEM

No Drawing. Application filed January 10, 1930, Serial No. 420,021, and in Germany January 21, 1929.

The present invention relates to the manufacture of alkyl-aralkyl-cellulose esters and to the new products obtainable thereby.

According to the process of my copending application Serial No. 331,952, filed January 11, 1929, the incompletely alkylated celluloses, containing  $\frac{1}{2}$  to  $1\frac{1}{2}$  alkyl groups calculated on one cellulose molecule and being soluble in water and alkalies, are subjected to acidylation, whereby alkyl cellulose esters are obtained in which about  $2\frac{1}{2}$  hydroxy groups, calculated on one molecule  $C_6H_{10}O_5$ , are substituted.

However, considerable difficulty arises in the technical execution of the process. The incompletely alkylated celluloses above characterized, of which, technically, only the methyl and ethyl celluloses are made use of, are very readily and usually completely soluble not only in cold water, but also in boiling water whereby they lose so much material (30% and more), that the process is rendered very expensive. Furthermore, when working on a technical scale, a partial cooling (for example cooling due to evaporation) can hardly be avoided. Before the alkylcelluloses are completely dry, they swell up under the influence of cold water, agglomerate or cake and then form lumps which are impermeable to the acidylating mixture. Thus, although the extraordinary ease with which the incompletely alkylated celluloses can be further acidylated, offers a great advantage, there is little success when carrying out the process on a large scale.

In accordance with the present invention, this disadvantage is overcome by esterifying with a fatty acid containing not more than 4 carbon atoms an incompletely alkylated cellulose containing in mixture a small amount of an aralkyl cellulose, such as benzyl cellulose, by acting upon said cellulose ether with the anhydride of the fatty acid to be introduced in the presence of the free fatty acid as solvent and of an acylation catalyst; for it has been found that the solubility in water or swelling power of the alkylcelluloses, containing  $\frac{1}{2}$  to  $1\frac{1}{2}$  mol of an alkyl group per one mol of  $C_6H_{10}O_5$  is eliminated, when the alkylcelluloses contain in admixture a small

percentage of aralkylcellulose, such as benzyl-, bromobenzyl-, nitrobenzyl- or toluyl-cellulose, a content of only  $\frac{1}{2}$ –2% of aralkyl cellulose being sufficient. It is immaterial whether the aralkyl ether is produced together with the alkyl ether in a single process, in which the etherifying agent introducing the aralkyl group, such as benzyl chloride, is added to the alkylating mixture, or whether the alkylating agent is caused to react on the finished, incompletely alkylated cellulose compound.

The amount of the aralkylating agent, such as benzyl chloride, to be added may range from  $\frac{1}{20}$  to  $\frac{1}{3}$  of one molecular proportion, advantageously being  $\frac{1}{5}$  of one molecular proportion, calculated on the  $C_6H_{10}O_5$  molecule. Taking into consideration the saponification of the aralkyl halogenide to the corresponding alcohol, there is obtained, for example, when using  $\frac{1}{5}$  of one molecular proportion of benzyl chloride, a mixed ether containing about 1% of benzyl cellulose. These methyl- or ethyl-aralkyl-celluloses are no longer soluble in water, with the result that they can be washed free from salts and alkalies without loss. For example, for 100 parts by weight of cellulose, 115 parts by weight of monethyl cellulose (containing about 1% benzyl cellulose) are obtained, while the calculated amount is 117 parts by weight. The swelling is so small even in ice water, that an agglomeration or sticking together of the swollen fibers no longer takes place and an easy penetration with the acetylating mixture is secured. The acidylation is not affected by the aralkyl content. In the alkyl-aralkyl-ester finally obtained the effect of the aralkyl content is shown by the decrease in the degree of swelling in water of, for example, a 1-ethyl- $1\frac{1}{2}$ -acetyl cellulose, containing about 1% of benzyl cellulose, falling from about 1.5% to less than 0.5%. With this is associated an excellent stability to boiling of the films and artificial threads prepared therefrom.

The invention is illustrated by the following example, but is not restricted thereto:

*Example.*—100 parts by weight of cellulose (cotton or wood pulp) are soaked with an

55

60

65

70

75

80

85

90

95

100

aqueous caustic soda solution of 30 per cent strength, pressed to 2½ times the above weight, mixed with 100 parts by weight of ethyl chloride and 14 parts by weight of 5 benzyl chloride (= ½ mol. calculated on  $C_6H_{10}O_5$ ) and heated for 3 hours at 110° C. The reaction product is washed free from salts and alkalies by means of water and dried. 115 parts by weight of a monoethyl 10 cellulose (containing about 1% benzyl) are obtained.

To 100 parts by weight of this monoethyl cellulose 160 parts by weight of acetic anhydride, 500 parts by weight of acetic acid and 15 1 part by weight of sulfuric acid are added and acetylation is effected with slow heating to 30° C. for two hours in a suitable apparatus. Thereupon the ether-acetate is precipitated directly with water without hydrolyzing and washed free from acid.

A monoethyl-1½-acetyl cellulose containing about 1% of benzyl cellulose, is obtained, which is soluble in acetone, acetic ester and chlorinated hydrocarbons and yields very 25 clear and strong films and is particularly suitable for the manufacture of artificial threads. The stability to water of the latter surpasses that of all other artificial silk materials.

30 I claim:

1. In the process of preparing alkyl-aralkyl-cellulose esters, the step which comprises esterifying by reacting with the anhydride of the fatty acid to be introduced in the 35 presence of the free fatty acid as solvent and of an acylation catalyst upon an alkyl-aralkyl-cellulose in which about ½-1½ hydroxy groups calculated on the molecule  $C_6H_{10}O_5$  are etherified and containing about 40 ½-2% of aralkyl-cellulose.

2. In the process of preparing alkyl-aralkyl-cellulose esters, the step which comprises esterifying by reacting with the anhydride of the fatty acid to be introduced in the 45 presence of the free fatty acid as solvent and of an acylation catalyst upon an alkyl-benzyl-cellulose in which about ½-1½ hydroxy groups calculated on the molecule  $C_6H_{10}O_5$  are etherified and containing about ½-2% of 50 benzyl-cellulose.

3. In the process of preparing alkyl-aralkyl-cellulose esters, the step which comprises esterifying by reacting with the anhydride of the fatty acid to be introduced in the 55 presence of the free fatty acid as solvent and of an acylation catalyst upon an ethyl-benzyl-cellulose in which about ½-1½ hydroxy groups calculated on the molecule  $C_6H_{10}O_5$  are etherified and containing about ½-2% of 60 benzyl-cellulose.

4. In the process of preparing alkyl-aralkyl-cellulose esters, the step which comprises acetylation by reacting with acetic anhydride in the presence of acetic acid and 5 an acetylation catalyst upon an alkyl-

aralkyl-cellulose in which about ½-1½ hydroxy groups calculated on the molecule  $C_6H_{10}O_5$  are etherified and containing about ½-2% of aralkyl-cellulose.

5. In the process of preparing alkyl-aralkyl-cellulose esters, the step which comprises acetylation by reacting with acetic anhydride in the presence of acetic acid and an acetylation catalyst upon an alkyl-benzyl-cellulose in which about ½-1½ hydroxy groups calculated on the molecule  $C_6H_{10}O_5$  are etherified and containing about ½-2% of benzyl-cellulose.

6. In the process of preparing alkyl-aralkyl-cellulose esters, the step which comprises acetylation by reacting with acetic anhydride in the presence of acetic acid and an acetylation catalyst upon an ethyl-benzyl-cellulose in which about ½-1½ hydroxy groups calculated on the molecule  $C_6H_{10}O_5$  are etherified and containing about 1% of benzyl-cellulose.

7. As new products alkyl-aralkyl-cellulose esters in which about 2½ hydroxy group calculated on the molecule  $C_6H_{10}O_5$  are substituted, obtainable in accordance with a process as claimed in claim 1, being generally soluble in acetone, acetic ester and chlorinated hydrocarbons and yielding very clear and strong films and artificial threads substantially stable to water.

8. As new products alkyl-benzyl-cellulose esters in which about 2½ hydroxy group calculated on the molecule  $C_6H_{10}O_5$  are substituted, obtainable in accordance with a process as claimed in claim 2, being generally soluble in acetone, acetic ester and chlorinated hydrocarbons and yielding very clear and strong films and artificial threads substantially stable to water.

9. As new products ethyl-benzyl-cellulose esters in which about 2½ hydroxy group calculated on the molecule  $C_6H_{10}O_5$  are substituted, obtainable in accordance with a process as claimed in claim 3, being generally soluble in acetone, acetic ester and chlorinated hydrocarbons and yielding very clear and strong films and artificial threads substantially stable to water.

10. As new products alkyl-aralkyl-cellulose acetates in which about 2½ hydroxy group calculated on the molecule  $C_6H_{10}O_5$  are substituted, obtainable in accordance with a process as claimed in claim 4, being generally soluble in acetone, acetic ester and chlorinated hydrocarbons and yielding very clear and strong films and artificial threads substantially stable to water.

11. As new products alkyl-benzyl-cellulose acetates in which about 2½ hydroxy group calculated on the molecule  $C_6H_{10}O_5$  are substituted, obtainable in accordance with a process as claimed in claim 5, being generally soluble in acetone, acetic ester and chlorinated hydrocarbons and yielding very clear and

strong films and artificial threads substantially stable to water.

12. As a new product an ethyl-benzyl-cellulose acetate in which about  $2\frac{1}{2}$  hydroxy groups calculated on the molecule  $C_8H_{10}O_5$  are substituted, obtainable in accordance with a process as claimed in claim 6, being generally soluble in acetone, acetic ester and chlorinated hydrocarbons and yielding very clear and strong films and artificial threads substantially stable to water.

In testimony whereof, I affix my signature.

ERNST TEUPEL. [L. S.]

15

20

25

30

35

40

45

50

55

60

65